

# UNITED STATES PATENT OFFICE.

PETER SCHMID AND KARL GROSS, OF BASEL, SWITZERLAND; SAID GROSS ASSIGNOR TO  
SAID SCHMID.

## PROCESS FOR THE MANUFACTURE OF A SUBSTITUTE FOR THE SERICIN SOAP FOR DYEING SILK, SILK-SPUNS, AND SILK TISSUES.

1,199,434.

Specification of Letters Patent. Patented Sept. 26, 1916.

No Drawing.

Application filed October 7, 1915. Serial No. 54,500.

To all whom it may concern:

Be it known that we, PETER SCHMID, a citizen of the Swiss Republic, and KARL Gross, a subject of the King of Prussia, both residing in Basel, Switzerland, have invented a new Process for the Manufacture of a substitute for the Sericin Soap for Dyeing Silk, Silk-Spuns, and Silk Tissues, of which the following is a full, clear, and

10 exact specification.

It is known, that for dyeing silk almost never is sericin soap at hand in sufficient quantities. For this reason many attempts have been made to utilize various substances 15 and preparations for producing artificial sericin soap; but until now no substitute of this kind has been found which would be able to replace the sericin soap produced by ungumming silk. We have now found, 20 that an excellent substitute for sericin soap can be obtained by boiling silkworm-chrysalises or silk-wastes containing silkworm-chrysalises, as for instance bassinets (Italian *gallettamini*, French *pelettes*). By preparing this substitute for sericin soap an alkali metal carbonate, as soda may be added to the water used, in order to saponify simultaneously the oils and greases contained in the chrysalises. The substitute for 25 sericin soap obtained according to the new process contains mainly substances approaching by their chemical compositions that of the sericin, whereby when using the same in dyeing, the touch, the luster, the elasticity and the strength of the fiber and 30 its regular coloration are influenced favorably.

Example: In a vat of 600 liters, provided with a steam coil and disposed above a reservoir containing 5000 liters pure water, are introduced 175 kg. bassinets and the vat is filled with pure water. The contents of the vat are constantly maintained warm by supplying steam to the coil. As soon as 40 the chrysalises dissolve, a little stream of the vat contents is allowed to flow through a cloth filter into the 5000 liters of water contained in the reservoir and by adding gradually bassinets into the vat the quantity of bassinets is continually maintained 45 in the vat in the same amount, and by a continual supplying of water the vat is

continually maintained filled with water. When the 5000 liters of water in the reservoir have received the boiled product resulting from the first 175 kg. bassinets, the contents of the said reservoir constitute a substitute for sericin soap having the same action as the usual sericin soap obtained by ungumming silk with 250 kg. soap. 55 60

In the foregoing example crystallized soda, for instance in proportion of 5 per cent. of the weight of the employed bassinets, can be added to the vat contents and in this case the vat contents can every day be 65 heated to ebullition for about  $\frac{1}{2}$  hour, whereby the oils and greases of the chrysalises are partly saponified.

What we claim is:

1. The described process for the manufacture of a substitute for sericin soap for dyeing silk, silk wastes, silk spuns and silk tissues, consisting in boiling silkworm-chrysalises with water. 70

2. The described process for the manufacture of a substitute for sericin soap for dyeing silk, silk wastes, silk spuns and silk tissues, consisting in boiling silkworm-chrysalises with water containing an alkali metal carbonate, in order to saponify 80 the oils and greases of the chrysalises. 75

3. The described process for the manufacture of a substitute for sericin soap for dyeing silk, silk wastes, silk spuns and silk tissues, consisting in boiling silk-wastes containing silkworm-chrysalises with water. 85

4. The described process for the manufacture of a substitute for sericin soap for dyeing silk wastes, silk spuns and silk tissues, consisting in boiling silk wastes containing silkworm-chrysalises with water containing an alkali metal carbonate, in order to saponify the oils and greases of the chrysalises. 90

In witness whereof we have hereunto signed our name this 14th day of September 1915, in the presence of two subscribing witnesses.

PETER SCHMID.  
KARL GROSS.

Witnesses:

ARNOLD ZUBER,  
AMAND RITTER.